

3,369,281

**STRETCH YARN MADE OF COTTON AND COTTON TYPE MATERIALS AND PROCESS OF PRODUCING THE SAME**

Georg Edlich, Lorrrach, Baden, Germany, assignor to Schipat AG, Zug, Switzerland, a corporation of Switzerland

No Drawing. Filed Oct. 1, 1965, Ser. No. 492,281  
Claims priority, application Germany, Oct. 15, 1964,  
E 27,959

8 Claims. (Cl. 28—76)

This invention relates to improvement in the qualities of so-called stretch yarn made of cotton and similar fibrous material.

Stretch yarn is generally understood by those skilled in the textile art to be a yarn material having permanent-elastic qualities which are not lost through subsequent after-treatment, such as, dyeing, washing, or the like, even without the application of tension. In the contrary, stretch yarns, even when processed provide garments which cling to the body, following its movements while retaining their original shape even under prolonged tensional and compressive stresses. Such stretch yarn commonly consists of synthetic fibers but is also known to be made of cotton. Such a stretch yarn made of cotton is prepared by first treating highly overtwisted yarns or twists under tension with humid heat, such as steam, and thereafter dyeing them again under tension.

It is also known to mercerize cotton yarns and fabrics, that is to treat them with aqueous alkaline solutions to shrink them and provide non-elastic crepe goods. Most recently there is also a process of mercerization which operates without tension and provides all-cotton stretch socks with qualities of clinging and relaxation which, however, do not equal those of texturized synthetic goods. This process consists in treating extremely loosely knitted socks without tension with rather concentrated sodium hydroxide lye, viz., 15—30%, at temperatures ranging between 26° and 91° C. It has been found that higher yarn twists, higher caustic concentrations and lower temperatures result in a reduction of the softness in hand. The yarns which were used had a normal twist and, in order to test yarns having an extreme twist (so twisted to avoid twisting of the goods during knitting), yarns were used which consisted of two yarns highly twisted in the same sense or direction and twisted together in the reverse sense.

According to the invention it has been unexpectedly discovered that the foregoing principle of slack mercerization also provides the desired stretch effect with extremely low lye concentrations if the yarn to be treated is given a specific twist structure. Such structure principally consists in the doubling of at least two single yarns having the same degree of twist but in opposite directions ("S" and "Z" twist), the doubling being in a greater measure than the twist of the single yarns.

Twists structured in this manner wherein the single yarn which untwists during the doubling embraces the other single yarn which overtwists during the doubling are known per se and for the most part consist of combinations of synthetic and natural yarns. Such twists are given some elastic stretchability by the overtwisted yarn component and softness in hand or velvet sheen by the embracing yarn. However, these known twists and textile goods made thereof have not been heretofore after-treated according to the principle of the slack mercerization.

It is accordingly a primary object of the present invention to provide an improved stretch yarn made of cotton and cotton type materials and a process of producing the same.

The present invention primarily comprises a cotton stretch yarn characterized in that it consists of at least two single yarns double with 136—166 turns per meter, each single yarn having the same degree of individual twist but of opposite direction or sense. The individual twist is weaker than the degree of double twist, such as 106—122 turns per meter, and the yarn is mercerized in hot 0.05% sodium hydroxide lye. The invention also comprises textile goods made of such stretch yarn.

10 The invention also comprises a process of producing such a cotton stretch yarn, such process being characterized in that at least two single yarns each being twisted with the same 106—122 turns per meter but in opposite direction or sense with respect to each other are doubled with a twist measure of 136—166 turns per meter, said measure being higher than that of the single yarn twists. The produced twist is mercerized in a hot about 0.05% caustic lye comprising a surfactant and afterwards is dried. Such mercerization may be given the non-fabricated twist as such but is preferably given the textile goods, e.g. the knitted or woven fabric. In both cases the treatment is performed with the twist in a non-tensioned state.

25 The surfactant, e.g. a conventional fat sulfonate, promotes the diffusion of the weak lye especially into the over-twisted core yarn whereby a cross-swell of the fibers and a corresponding longitudinal shrinking of the fabric is caused and fixed by the subsequent drying. The finished yarn and the textile goods produced therefrom have a high elastic elongation of 30—40% together with softness in hand and luminous or bulky appearance.

30 As used herein the term "caustic lye" comprises all substances which react in a mercerizing manner on cotton, viz., causing a shrinking of its fibers. In the interest of economy and easy availability a commercially available sodium hydroxide lye of about 41.65% NaOH contents is used and applied in a concentration of 0.1%. As used herein the term "cotton" comprises cotton as such as well as all synthetic and natural substances which by reaction with weak alkaline solutions undergo a swelling which is stable even on subsequent washing or other finishing processes of the fiber substance of the threads, such swelling being accompanied by a longitudinal shrinkage of the fibers. Such substances are known to those skilled in the mercerization art. Cotton per se and such cotton type materials are referred to collectively as cotton type materials in the claims herein. As used herein the term "hot" (lye) used for characterizing the invention comprises the area of temperature adjacent to the boiling point of the lye and is inversely reciprocally related to the duration of treatment in the manner known for chemical reactions. According to experience a one hour treatment with a 0.1% sodium hydroxide lye at about 85° provides for the desired stretch yarn effect.

55 From the preceding it is evident that the invention consists of a combination of—on the one hand—a mechanical treatment (twisting) and—on the other hand—a chemical treatment (mercerization), both treatments being individually specific and harmonized with one another. In comparison with known methods there is no use of any twist or rippling. By the omission of any fixation whatsoever by synthetic resin and by the use of extremely weak lye concentrations essential savings in material costs are achieved. Furthermore, operation with such weak lyes eliminates the serious problem of accident prevention, otherwise encountered with the use of lyes, and effects a reduction of operational costs by eliminating the otherwise necessary washing of the final fabric to remove the lye.

70 Through the invention there is provided the substantial advantage that both the stretch yarn, as such, and

the textile goods produced therefrom, retain the natural qualities of the starting material e.g. cotton, such as heat retention, air permeability, ability to take up moisture, resistance to abrasion, and softness of fibers, and the final textile goods, especially as a shaped garment, have a permanent stretchability of 30-40% as a knitted or woven product, and additionally are of permanent shape and resistant to creasing.

The following examples are intended as illustrative only, it being understood that the invention is not restricted thereto, it being evident that the invention may be realized in a variety of other ways within the scope of the invention and appended claims.

#### EXAMPLE 1

Links-links fabrics produced on a 22-inch circular links- and links machine provided with 12 needles per inch; adjustment=95 mm./100 links (measured in the area between needle bed and stripping comb), that is, the fabric is measured in tensioned state within the machine for determining the adjustment.

*Fabric A* made of stretch Ne 30/2 cotton yarn (according to the invention).

*Fabric B* made of normal Ne 30/2 cotton yarn.

The following values were taken from the relaxed fabric, viz, after resaturation of the balance of the loop forces by wet treatment at elevated temperatures:

|                                       | A   | B   |
|---------------------------------------|-----|-----|
| Width of the hose, mm.....            | 500 | 580 |
| Weight per square meter, g.....       | 220 | 150 |
| Cross elongation, percent.....        | 49  | 40  |
| Longitudinal elongation, percent..... | 131 | 115 |

#### EXAMPLE 2

*1.1 knitted fabric* (rechts-and-rechts-fabric with alternating rechts-and-links-wales) produced on a 15-inch circular machine provided with 18 needles per inch; adjustment=90 mm./100 links (measured as in Example 1).

*Fabric A* made of stretch Ne 70/2 cotton yarn (according to the invention).

*Fabric B* made of normal Ne 35/1 cotton yarn.

Values of the fabrics relaxed as in Example 1:

|                                       | A   | B   |
|---------------------------------------|-----|-----|
| Width of the hose, mm.....            | 420 | 420 |
| Weight per square meter, g.....       | 178 | 142 |
| Cross elongation, percent.....        | 31  | 17  |
| Longitudinal elongation, percent..... | 136 | 175 |

The higher value of longitudinal elongation of B is caused by the lower adjustment and mostly consists of permanent undesired elongation.

The invention may be embodied in other specific forms without departing from the spirit or essential characteristics thereof. The present embodiments are therefore to

be considered in all respects as illustrative and not restrictive, the scope of the invention being indicated by the appended claims rather than by the foregoing description and all changes which come within the meaning and range of equivalency of the claims are therefore intended to be embraced therein.

What is claimed and desired to be secured by United States Letters Patent is:

1. A process of producing a stretch yarn of a mercerized cotton type material, comprising the steps of forming at least two individual yarns each having substantially the same twist of 106-122 turns per meter but of opposite sense with respect to one another, twisting said individual yarns together with a twist of 136-166 turns per meter which is higher than that of the individual yarns, mercerizing the produced twist in a hot caustic lye of about 0.05% comprising a surfactant, and drying.
2. A process as claimed in claim 1, wherein the caustic lye comprises a 0.01% sodium hydroxide lye having a temperature of about 85° C.
3. A process of producing a textile fabric of mercerized cotton stretch yarn, comprising the steps of forming at least two individual yarns each having the same twist of 106-122 turns per meter but of opposite sense with respect to one another, twisting said individual yarns together with a twist of 136-166 turns per meter which is higher than that of the individual yarns, forming a body of links from the produced twist, mercerizing the produced body of links in a hot caustic lye of about 0.05% comprising a surfactant, and drying the body of links.
4. A process as claimed in claim 3, wherein the caustic lye comprises a 0.01% sodium hydroxide lye having a temperature of about 85° C.
5. A process as claimed in claim 4 including the step of forming said fabric into a shaped garment.
6. A process as claimed in claim 3 including the step of forming said fabric into a shaped garment.
7. A stretch yarn made according to the process of claim 1.
8. A fabric made according to the process of claim 3.

#### References Cited

##### UNITED STATES PATENTS

|           |         |                               |
|-----------|---------|-------------------------------|
| 8,303     | 8/1851  | Mercer.                       |
| 1,885,019 | 10/1932 | Theis _____ 28-76             |
| 2,153,963 | 4/1939  | Lejeune et al. _____ 28-76 XR |
| 2,153,964 | 4/1939  | Lejeune _____ 28-76 XR        |
| 3,127,732 | 4/1964  | Brown et al. _____ 57-164     |
| 3,132,497 | 5/1964  | Garrou _____ 66-202           |
| 3,145,132 | 8/1964  | Seltzer _____ 28-76 XR        |
| 3,287,788 | 11/1966 | Goodbar et al. _____ 28-76    |
| 3,299,486 | 1/1967  | Meyers et al. _____ 28-76     |

FRANK J. COHEN, Primary Examiner.

J. PETRAKES, Examiner.